

1

2,894,828

## HYDROCARBON COMPOSITIONS CONTAINING THE WATER-INSOLUBLE NITRIC ACID OXIDATION PRODUCT OF NAPHTHENIC ACIDS

Peter B. Kelly, College Station, Tex., assignor to Gulf Research &amp; Development Company, Pittsburgh, Pa., a corporation of Pennsylvania

No Drawing. Application March 15, 1956  
Serial No. 571,608

5 Claims. (Cl. 44—72)

This invention relates to anti-rust agents for hydrocarbon compositions and hydrocarbon compositions containing the same, and more particularly, it relates to hydrocarbon compositions containing the water-insoluble nitrogen-containing product resulting from the oxidation of a naphthenic acid with nitric acid.

Rusting of ferrous metals due to the presence of water as a contaminant in some hydrocarbon compositions is a serious problem in the storage, handling and use of such compositions. Although gasoline, oil and other hydrocarbons derived from petroleum are substantially free from moisture when they leave the refinery, traces of water may later be found in these products. Liquid petroleum products are frequently removed from storage tanks by water displacement, thus giving rise to the possibility of water contamination. In other instances, water can be introduced into petroleum products through faulty tank closures. Storage tanks for petroleum hydrocarbons because of their volatility must be constructed to allow room for expansion and must be provided with adequate breathing devices. Thus, as the contents of the tank contract, at night, for example, moist air is drawn in. The moisture thus drawn in condenses and settles to the bottom of the tank. The next day as the tank heats up the contents of the tank expand thus forcing out dried air. As this cycle is repeated day after day, appreciable amounts of water are collected in the bottom of the tank. Water contamination is particularly a problem in humid atmospheres such as those encountered in the tropics and on the seaboard as well as onboard ships.

In accordance with the present invention, a hydrocarbon composition is provided which gives prolonged protection against rusting normally resulting when metals are exposed to hydrocarbon compositions containing water as a contaminant.

I have discovered that a hydrocarbon composition can be improved with respect to its anti-rust characteristics by incorporating in said hydrocarbon composition a small amount of the water-insoluble nitrogen-containing reaction product obtained by contacting a naphthenic acid under oxidizing conditions with nitric acid. My invention, based on this discovery, thus comprises a hydrocarbon composition containing an anti-rust improving amount of the water-insoluble nitrogen-containing reaction product obtained by contacting a naphthenic acid under oxidizing conditions with nitric acid.

The hydrocarbon compositions to which the anti-rust agent can be added in accordance with the invention can vary in volatility from light gasoline to heavy oils and greases. Within this volatility range I intend to include diesel fuels, lubricating oils, slushing oils, turbine oils, transformer oils, and the like. The gasoline can be a synthetic gasoline, a straight-run gasoline, a cracked gasoline, or blends thereof, and it can contain components obtained from processes other than cracking, such as components obtained from alkylation, isomerization, hydrogenation, polymerization, hydrodesulfurization, hy-

2

droforming, "Platforming," or combinations of two or more such processes.

When the hydrocarbon composition to which the anti-rust agent is added is gasoline the gasoline can contain minor amounts of addition agents other than the anti-rust agent of the invention. Thus for example, the gasoline can contain octane improving amounts of tetraethyl lead fluid. Other addition agents normally added to gasolines for a specific purpose such as an anti-oxidant, a haze inhibitor, an oiliness agent, an anti-stalling agent, a corrosion inhibitor, a lead scavenging agent, a dye, etc., can be employed without adversely affecting the improved anti-rust characteristics derived in accordance with the invention.

When the hydrocarbon composition to which the anti-rust agent added is a lubricating oil the oil can be any oil having a viscosity within the range of common lubricating oils. The oil can be a synthetic oil or a mineral oil including refined or semi-refined paraffinic, naphthenic or asphalt base oil having a viscosity of about 50 to about 4000 SUS at 100° F. If desired, the anti-rust agent can be added to a blend of oils of suitable viscosity instead of a single oil by means of which any desired viscosity within the range of 50 to 4000 SUS at 100° F. can be secured.

When a lubricating composition is desired the lubricating oil can contain minor amounts of an addition agent other than the anti-rust agent of the invention. Thus for example, it is particularly advantageous in many instances to add an anti-foam agent to the lubricating composition. Other addition agents normally added to lubricating oils for a specific purpose such as an anti-oxidant, pour point depressant, corrosion inhibitor, viscosity index improver, oiliness and extreme pressure agent, and the like, can be employed without adversely affecting the improved anti-rust characteristics derived by the composition of this invention.

When a naphthenic acid is oxidized in the presence of a strong oxidant such as nitric acid, chromic acid or potassium permanganate, the resulting reaction mass comprises a water-soluble portion and a water-insoluble portion. The water-soluble portion comprises dibasic carboxylic acids. When nitric acid is used as the oxidant, the water-insoluble portion comprises certain nitrogen-containing hydrocarbons, the exact structural formula of which has not been completely determined. The nitrogen content of the water-insoluble reaction product thus obtained comprises about 3 to about 6 percent by weight of the reaction product. The nitrogen substituted compounds thus obtained when present in petroleum hydrocarbons, even in exceedingly small amounts, have the property of inhibiting the rusting of iron and steel surfaces.

The process of oxidizing a naphthenic acid in the presence of nitric acid can be readily effected at atmospheric pressure at a temperature between about 70° and about 120° C. While it is preferred to carry out the reaction at atmospheric pressure, the reaction can also be carried out at elevated pressures in the order of about 1000 pounds per square inch gauge. As the pressure is raised the reaction temperature can correspondingly be raised to about 150° C.

The concentration of the nitric acid employed in the oxidation of the naphthenic acid is not critical, although it should be high enough to convert a substantial amount of the naphthenic acid to a dibasic carboxylic acid in a reasonable length of time. Thus, the concentration of the nitric acid can be as low as about 30 percent or as high as about 100 percent, although a concentration of about 70 percent is generally preferred.

The ratio of nitric acid to naphthenic acid is not critical, although an amount of nitric acid in excess of that

theoretically required to oxidize the naphthenic acid in the charge to a dibasic carboxylic acid is preferred. In general, a ratio of at least about two parts, and preferably at least about four parts, of nitric acid per part of naphthenic acid is satisfactory.

The time required for the substantial completion of the reaction will depend, of course, upon the selection of variables defined hereinabove. Since the reaction is exothermic, from a practical point of view the time required will depend, to a large part, upon the rate at which heat produced can be removed from the reaction system. A period of at least about  $\frac{1}{2}$  hour and preferably about 1 to about 100 hours is generally satisfactory to convert a naphthenic acid to the corresponding dibasic carboxylic acid. Simultaneously with this reaction water-insoluble nitrogen-containing hydrocarbons are formed. It is the latter products with which this invention is concerned.

The naphthenic acids which can be employed as the starting material to produce water-soluble dibasic acids and water-insoluble nitrogen-containing products can be defined as cycloparaffinic compounds containing at least one carboxylic acid group per molecule, particularly those whose boiling points range from about 390° to about 660° F., and whose molecular weights are about 128 to about 480. As charge stock in producing the useful additive for the invention, any of the naphthenic acids defined above or mixtures of such naphthenic acids can be employed. Preferably, the charge stock consists almost solely of naphthenic acids, although minor amounts of other closely associated compounds or materials which do not adversely affect the course of the oxidation reaction can be present. Included among the naphthenic acids which are suitable starting materials in producing the water-insoluble product for use in the invention are methylcyclopentane carboxylic acid, dimethylcyclopentane carboxylic acid, methylcyclohexyl carboxylic acid, methylcyclohexyl acetic acid, etc. Commercially available mixtures of naphthenic acids can be used in accordance with the invention. Of the commercially available naphthenic acids, I prefer the  $C_8$  to  $C_{12}$  acids. However, higher molecular weight acids, i.e., those containing more than 12 carbon atoms including those having double naphthenic rings can be used.

The oxidizing action necessary to produce appreciable yields of water-soluble dibasic acids and water-insoluble nitrogen-containing compounds must be strong and therefore mere air blowing will not suffice, although an oxygen-containing gas such as air in combination with nitric acid can be employed to reduce the consumption of nitric acid. In such a case an amount of air to give 100 percent by weight of molecular oxygen based upon the nitric acid can be employed. While any strong oxidant can be used where the sole desired product is a dibasic carboxylic acid, only nitric acid can be used to give the desired water-insoluble nitrogen-containing compound employed in accordance with this invention. The oxidation of naphthenic acids to produce the water-insoluble nitrogen-containing product employed in accordance with the invention can be conducted with or without the aid of an oxidation-promoting catalyst. Included among the oxidation-promoting catalysts which can be used are ammonium metavanadate, potassium permanganate and cobalt nitrate.

The optimum amount of reaction product employed in any given material will vary somewhat depending upon the particular hydrocarbon composition employed and upon the severity of the rust-inducing conditions encountered. The amount of the water-insoluble nitrogen-containing reaction product employed in a liquid hydrocarbon composition can comprise about 1 to about 20 pounds per thousand barrels of hydrocarbon. When the hydrocarbon composition is gasoline, I have obtained highly satisfactory anti-rust characteristics when the water-insoluble nitrogen-containing reaction product was employed in amounts of from 5 to 15 pounds per thousand barrels.

In any event, I employ an amount of the water-insoluble nitrogen-containing reaction product sufficient to inhibit or substantially prevent the rusting of ferrous metal surfaces normally encountered when the hydrocarbon composition contains no such reaction product. I have found that the incorporation of this reaction product in gasoline in amounts of from 5 to 15 pounds per thousand barrels has no deleterious affect on the other desirable characteristics of the fuel.

The following examples will illustrate the preparation of compounds useful in my invention.

#### EXAMPLE 1

Four hundred grams of petroleum naphthenic acids having a boiling range of about 100° to about 125° C. at 2.5 mm. of Hg and a molecular weight of 220 was added dropwise to 1600 ml. of 70 percent nitric acid containing one gram of ammonium metavanadate. The mixture thus formed was stirred and heated to 85° C. This temperature was maintained ( $\pm 5^\circ$  C.) until substantially all of the hydrocarbon layer had disappeared. The reaction mixture was then cooled whereupon the mixture formed a hydrocarbon layer and an aqueous layer. The aqueous layer containing a substantial portion of the nitric acid was removed and further processed to recover polybasic acids. The hydrocarbon layer was dissolved in twice its volume of benzene and then washed with water until the water used for washing was colorless. The benzene layer was then dried over calcium chloride and the benzene removed by vacuum distillation. The product thus obtained was the water-insoluble nitrogen-containing product useful as an anti-rust agent according to my invention. The product was a clear, reddish oil with a disagreeable odor. This product had a carbonyl number of 90.3, a saponification number of 410 and a molecular weight of 226. The oxidized product contained 58.76 percent carbon, 7.95 percent hydrogen, 5.47 percent nitrogen and 24.82 percent oxygen (by difference).

#### EXAMPLE 2

Fifty grams of petroleum naphthenic acids having a boiling range of about 50° to about 160° C. at 2 mm. of Hg and a neutralization value of 158 was oxidized as in Example 1 using 200 ml. of 35 percent nitric acid containing 0.2 gram of ammonium metavanadate. The product obtained after heating the mixture at 85° C. as in Example 1 consisted of two layers which were separated by decantation. The lower aqueous layer was further processed to recover polybasic acids. The hydrocarbon layer was dissolved in toluene and then washed with water until the wash water was colorless. The toluene layer was then dried over calcium chloride and the toluene removed by vacuum distillation. The dried product thus obtained was the water-insoluble nitrogen-containing product useful as an anti-rust agent according to my invention. This product had a neutralization value of 141 and a nitrogen content of 3.4 percent.

In order to illustrate the improved anti-rust characteristics obtained with a gasoline containing the water-insoluble reaction product obtained in Example 1, such a gasoline has been compared with a gasoline containing no anti-rust agent, with a gasoline containing a commercially available anti-rust agent, and with a gasoline containing unoxidized naphthenic acids. The unoxidized naphthenic acids used for comparison were those used in preparing the water-insoluble nitrogen-containing reaction product of Example 1. The comparison was made by placing 6" x  $\frac{3}{4}$ " SAE 1020, sand blasted, solvent rinsed steel strips in contact with mixtures of water and gasoline for prolonged periods of time. The steel strips were then examined for rust formation. In making the determinations, 400 ml. of gasoline and 100 ml. of distilled water were placed in a glass container. Steel strips were placed in the container so that part of each

strip was in the water layer, another part in the gasoline layer, and a further part in the air space above the liquid. The container was tightly sealed and then violently agitated for about 1 minute. The container was then stored in the dark at room temperature without further agitation. Steel strips were removed from the container at different intervals to determine the amount of rust formed on the various segments. Steel specimens which were completely free from rust were given an anti-rust rating of 100. Steel strips which were completely covered with rust were given an anti-rust rating of zero.

Table I summarizes the results obtained with gasoline containing various additives in concentrations as shown.

Table I

| Additive               | Concentration, lb./1,000 bbl. | Anti-rust Rating Time in Hours |     |      |     |
|------------------------|-------------------------------|--------------------------------|-----|------|-----|
|                        |                               | 0                              | 24  | 142  | 162 |
| None                   |                               | 100                            | 44  | 38   | 35  |
| Do                     |                               | 100                            | 146 | 233  | 33  |
| Commercially available | 10                            | 100                            | 85  | 70   | 70  |
| Do                     | 15                            | 100                            | 194 | 272  | 70  |
| Naphthenic acids       | 15                            | 100                            | 50  | 37   | 34  |
| Product of Example 1   | 5                             | 100                            | 93  | 81   | 78  |
| Do                     | 15                            | 100                            | 100 | 2100 | 93  |

<sup>1</sup> 3 hours.

<sup>2</sup> 113 hours.

<sup>3</sup> 161 hours.

The improved results obtained in accordance with my invention are apparent from the summary of data in Table I. It will be noted that the base gasoline and the gasoline containing naphthenic acids gave very little protection against rusting. However, the nitric acid oxidation product of Example 1 gave prolonged protection at concentrations of 5 to 15 pounds per thousand barrels of gasoline. The protection thus obtained was greater than that obtained with the commercially available additive in concentrations of 10 and 15 pounds per thousand barrels of gasoline.

The physical characteristics of gasoline are not substantially changed by the addition of the water-insoluble nitric acid oxidation product as evidenced by the following data.

| Test                                        | Gasoline | Gasoline+10 lb./1,000 bbl. Product of Example 1 |
|---------------------------------------------|----------|-------------------------------------------------|
| Existent Gum, mg./100 ml.                   | 2.7      | 5.0                                             |
| Copper Dish Gum, ASTM D910-52T, mg./100 ml. | 22       | 25                                              |
| Oxidation Stability, 212° F., min.          | 457      | 532                                             |
| Copper Strip Test, 122° F., 3 hr.           | Blank    | Blank                                           |
| Knock Rating:                               |          |                                                 |
| Research Method                             | 92.0     | 92.0                                            |
| Motor Method                                | 83.2     | 82.8                                            |

It will be noted that the oxygen stability of the gasoline is improved but that otherwise there is very little effect on the physical characteristics of the gasoline. While there appears to be a slight increase in the existent gum and in the copper dish gum, the increase is not actual gum formation but is due to the additive itself, which being non-volatile, remains as a residue when the gasoline is evaporated. In each instance, the additive amounts to about 2.8 mg. per 100 ml. of gasoline.

While my invention is described above with reference to various specific examples and embodiments, it will be

understood that the invention is not limited to such examples and embodiments and may be variously practiced within the scope of the claims hereinafter made.

I claim:

1. A hydrocarbon composition comprising a major amount of a normally liquid hydrocarbon normally tending to rust ferrous metals when contaminated with water and a small amount, sufficient to substantially retard such rusting, of the water-insoluble nitrogen-containing reaction product obtained by oxidizing at about 70° to about 150° C. one part by weight of a naphthenic acid having a boiling range of about 390° to about 660° F. at atmospheric pressure and a molecular weight of about 128 to about 480 in the presence of at least two parts by weight of nitric acid having a concentration of about 30 to about 100 percent, the oxidizing period being sufficient to produce a water-soluble dibasic carboxylic acid and said water-insoluble nitrogen-containing reaction product.
2. A hydrocarbon composition comprising a major amount of a normally liquid hydrocarbon normally tending to rust ferrous metals when contaminated with water and a small amount, sufficient to substantially retard such rusting, of the water-insoluble nitrogen-containing reaction product obtained by oxidizing at about 70° to about 150° C. one part by weight of a naphthenic acid having a boiling range of about 390° to about 660° F. at atmospheric pressure and a molecular weight of about 128 to about 480 in the presence of at least two parts by weight of nitric acid having a concentration of about 30 to about 100 percent, the oxidizing period being sufficient to produce a water-soluble dibasic carboxylic acid and said water-insoluble nitrogen-containing reaction product comprising about 3 to about 6 percent by weight of the reaction product.
3. A hydrocarbon composition having improved anti-rust characteristics which comprises a normally liquid hydrocarbon and about 1 to about 20 pounds per thousand barrels of said normally liquid hydrocarbon of the water-insoluble nitrogen-containing reaction product obtained by oxidizing at about 70° to about 150° C. one part by weight of a naphthenic acid having a boiling range of about 390° to about 660° F. at atmospheric pressure and a molecular weight of about 128 to about 480 in the presence of at least two parts by weight of nitric acid having a concentration of about 30 to about 100 percent, the oxidizing period being sufficient to produce a water-soluble dibasic carboxylic acid and said water-insoluble nitrogen-containing reaction product, the nitrogen content of said water-insoluble nitrogen-containing reaction product comprising about 3 to about 6 percent by weight of the reaction product.
4. A motor fuel having improved anti-rust characteristics which comprises a major amount of gasoline and about 5 to about 15 pounds per thousand barrels of gasoline of the water-insoluble nitrogen-containing reaction product obtained by oxidizing at about 70° to about 150° C. one part by weight of a naphthenic acid having a boiling range of about 390° to about 660° F. at atmospheric pressure and a molecular weight of about 128 to about 480 in the presence of at least two parts by weight of nitric acid having a concentration of about 30 to about 100 percent, the oxidizing period being sufficient to produce a water-soluble dibasic carboxylic acid and said water-insoluble nitrogen-containing reaction product, the nitrogen content of said water-insoluble nitrogen-containing reaction product comprising about 3 to about 6 percent by weight of the reaction product.
5. A motor fuel having improved anti-rust characteristics which comprises a major amount of gasoline and about 5 to about 15 pounds per thousand barrels of gasoline of the water-insoluble nitrogen-containing reaction product obtained by oxidizing at about 80° to about 90° C. one part by weight of petroleum naphthenic acids, having a boiling range of 100° to 125° C. at 2.5 mm. of

Hg and a molecular weight of about 220, in the presence of at least two parts by weight of nitric acid having a concentration of 70 percent and ammonium metavanadate, the oxidizing period being sufficient to produce a water-soluble dibasic carboxylic acid and said water-insoluble nitrogen-containing reaction product, the nitrogen content of said water-insoluble nitrogen-containing reaction product comprising about 5.5 percent by weight of the reaction product.

## References Cited in the file of this patent

## UNITED STATES PATENTS

- |           |                         |               |
|-----------|-------------------------|---------------|
| 2,196,101 | Carmichael et al. _____ | Apr. 2, 1940  |
| 2,401,993 | Wasson et al. _____     | June 11, 1946 |
| 2,478,243 | Coe et al. _____        | Aug. 9, 1949  |

## FOREIGN PATENTS

- |         |               |               |
|---------|---------------|---------------|
| 743,909 | Germany _____ | Nov. 11, 1943 |
|---------|---------------|---------------|